

Dec. 1, 1936.

C. H. VAN DUSEN, JR., ET AL

2,062,486

METHOD OF MAKING PYROPHORIC FLINTS

Filed April 27, 1934



FIG. 1.



FIG. 2

FIG. 3



FIG. 4

JINVENTOR  
CHARLES H. VAN DUSEN, JR.  
EDWIN C. DIETRICH  
Kris, Hudson & Kent  
ATTORNEYS

Patented Dec. 1, 1936

2,062,486

# UNITED STATES PATENT OFFICE

3,062,486

## METHOD OF MAKING PYROPHORIC FLINTS

Charles H. Van Dusen, Jr., Cleveland Heights, and Edwin C. Dietrich, East Cleveland, Ohio, assignors, by mesne assignments, to Cooper Sparkelite, Ltd., Dover, Del., a corporation of Delaware

Application April 27, 1934, Serial No. 722,692

### 8 Claims. (Cl. 29—148)

The present invention relates to the fabricating or working of pyrophoric alloys such as cerium and mischmetal alloys, and more particularly to composite flints made of these alloys, and a method of manufacturing the same.

In the familiar cigar and cigarette lighters of commerce, small pieces of pyrophoric alloys, commercially known as flints, are struck by suitably constructed toothed wheels or sharp rods, and give off sparks which usually ignite a suitably placed impregnated wick. These flints are usually rods or sticks of very small cross section and comparatively short length, and since the pyrophoric materials used are hard and brittle, it is impossible to convert them to the desired shape by the usual means of cold working such as hammering, rolling, drawing or swaging, etc. On the other hand, hot working is likewise impossible because of the great chemical activity of the material.

An object of the present invention is the provision of a novel commercial method of manufacturing, fabricating, or working pyrophoric alloys into useful shapes.

Another object of the invention is the provision of a novel commercial method of manufacturing flints of pyrophoric material which consists in working pyrophoric alloys within a protective metallic sheath to a desired shape and subsequently removing a portion of the protective metallic sheath to expose the pyrophoric alloy.

Further objects and advantages of the invention will be apparent to those skilled in the art to which it pertains from the following description of the preferred embodiment of the invention described with reference to the accompanying drawing, of which

Fig. 1 is an elevation of an ingot comprising a pyrophoric material enclosed in a protective sheath, with a portion of the sheath broken away to show the pyrophoric material;

Fig. 2 is a section of composite rod produced by the reduction of the ingot shown in Fig. 1;

Fig. 3 is a perspective of a composite flint embodying the present invention; and

Fig. 4 is a perspective of a lighter embodying the present invention.

According to the present invention, pyrophoric material, such as alloys of cerium or mischmetal, with iron, copper, nickel, zinc, or magnesium, etc., is enclosed in a protective metallic sheath and worked, usually by a plurality of successive steps, to the desired shape, after which the protective material is removed to expose the pyrophoric material. We have found that pyrophoric material lends itself readily to working and change of shape when it is properly supported on all sides, as is the present instance. This is especially true when the composite article is

worked at moderate temperatures or periodically annealed during the process of reduction. In addition to confining the metal so that it cannot separate while being worked, the protective metal sheath prevents the same from burning, and chemical reaction.

While individual articles of any size or shape may be made it has been found advantageous to make a rod of considerable length and subsequently cut the same to desired lengths. Preferably the pyrophoric alloy is first cast in rods of comparatively large cross section and suitable length, and slipped into a snugly fitting metallic tube, slightly longer than the rod, after which the ends of the tube are closed in any suitable manner, as by burnishing, spinning, swaging or hammering, etc., to form a composite rod or ingot. The composite rod or ingot is then rolled, drawn, swaged, or hammered etc., to form a rod of the desired cross-section or shape. The ingot or rod may be worked at a moderate temperature or may be annealed between passes or operations. The amount of work, that is, the percentage of reduction of cross section that is done at each pass through the hammer, rolls, swager, dies, or the like, is about the same as that with iron, copper or any ordinarily malleable metal. The protective sheath is then removed from the reduced composite rod to expose the pyrophoric material, by grinding, milling or planing, etc., after which the bar is cut to the desired lengths.

Referring to the drawing, Fig. 1 illustrates a composite rod or ingot formed of a round cast rod 10 of pyrophoric material, such as ferrocerium or ferro-mischmetal, enclosed in a snugly fitting tube or sheath 11 made of copper or other suitable metal, the ends 12 and 13 of which have been tightly closed in some convenient manner. The rod 10 illustrated is about one-half inch in diameter and ten or twelve inches long, and the copper tube or sheath 11 has a wall thickness of about one-sixteenth or three-thirty-seconds of an inch. The composite rod or ingot is reduced to the desired cross section or shape which in the present instance is illustrated in Fig. 2 as square, either by cold working, such as drawing, rolling etc., including inter-pass or inter-operation annealing, or by hot working at a temperature not to exceed 500° C. or a dull red heat. In the latter instance, as the cross-sectional area of the rod is decreased the working temperature may be rapidly reduced, and inter-pass or inter-operation anneals substituted for hot working. As the rod approaches the finished size the last few passes may be made without annealing which usually also increases the strength of the enclosing or supporting sheath.

After a composite rod of the desired cross section has been formed, which in the present instance is about one-eighth or five thirty-seconds

of an inch square, the enclosing sheath 11 is removed from one side thereof by passing the bar under a grinding wheel, etc., to expose the pyrophoric material. The sheath 11 supports the 5 pyrophoric material which is quite brittle, in such a manner that the reduced bar may be cut with a shears, punch press, etc., without cracking or crumbling. A length cut from the bar in this condition forms a composite flint A, illustrated in 10 Fig. 3, of the type adapted to be struck with a striking or scratch pin.

Flints of the present invention show a marked 15 superiority of pyrophoric properties over those of the prior art, and are more resistant to deterioration due to oxidation, etc., caused by exposure to air, moisture, carbon dioxide, etc., because a greater part of the surface is protected by a tightly adhering protective sheath. The stream 20 of sparks which are struck from the pyrophoric material, in operation, consists of small particles of metal which are torn off by the striker bar or toothed wheel. These small particles of metal are heated by the friction incident to the striking 25 or scratching and burn as they fly into the air. The superiority of the pyrophoric properties of 30 the present flint may be caused by the fact that apparently the working of the alloy produces a granular structure from which particles may be readily torn off by the striker bar.

While the specific embodiment of the invention 35 illustrated shows copper as the supporting material, it is to be understood that metals such as iron, nickel, aluminum, tin, silver, or any other metal or alloy having sufficient strength and 40 ductility, and a high enough melting point, may be substituted for the copper shown. It is also to be understood that while the copper sides are shown as being flush with the exposed surface of 45 the pyrophoric material, they may project above the exposed surface or any configuration of surface may be exposed.

Fig. 4 illustrates the flint shown in Fig. 3 embodied in a cigar or cigarette lighter B of the scratch pin type and conventional construction. 50 The flint A is embedded in the body of the lighter in any well known manner. As the exposed surface of the pyrophoric material wears down, the copper walls on the two sides act as guides for the striker or scratch pin and insure proper and 55 successful action at each stroke. With the contact of the striker against the pyrophoric material insured, a smaller or narrower surface of pyrophoric material is required, with consequent economy in the amount of material used. It will 60 be obvious that the cross section of the finished flint may be round as well as rectangular. In the manufacture of flints for use with toothed wheels it may be unnecessary to remove the protective covering as a separate operation since the pyrophoric material will be exposed at the ends upon the cutting of the reduced bar into the desired 65 lengths.

From the foregoing description of the invention, it will be apparent that a novel flint has been produced, together with a novel lighter and a novel 70 method of working pyrophoric material and manufacturing flints therefrom. It is not intended to be limited to the particular construction or method illustrated and described, as various changes therein may be made within the scope of the invention, but it is the intention to cover any and all variations, adaptations or uses thereof as

come within the knowledge or customary practice in the art to which this invention belongs, and we particularly point out and claim as our invention the following:

We claim:

1. The method of making a composite article of pyrophoric material and a protective metal covering a portion thereof, which comprises enclosing a pyrophoric alloy in a metallic sheath to form a composite ingot, reducing said ingot to the 10 desired shape, and subsequently exposing a portion of the pyrophoric alloy.

2. The method of making a composite flint of pyrophoric material and a metallic protective coating, which comprises enclosing the pyrophoric material in a metallic sheath, working the article thus formed to a desired shape, and subsequently removing a portion of the protective coating to expose the pyrophoric material.

3. The method of making a composite flint of pyrophoric material and a metallic covering which comprises enclosing the pyrophoric material in a metallic sheath to form an ingot, reducing said ingot by a hot metal working process to form a rod of desired shape, and subsequently removing a portion of the enclosing sheath from the rod to expose the pyrophoric material.

4. The method of making a composite flint of pyrophoric material and a metallic protective covering which comprises enclosing the pyrophoric material in a metallic sheath to form an ingot, reducing said ingot by a metal drawing process to form a rod of desired shape, and subsequently removing a portion of the protective coating to expose the pyrophoric material.

5. The method of making a composite flint of a pyrophoric alloy and a metallic covering which comprises casting the pyrophoric alloy into the form of a rod, enclosing the cast rod in a snugly fitting metallic sheath to form a composite ingot, reducing the composite ingot to a desired shape, and subsequently removing a portion of the enclosing sheath to expose the pyrophoric material.

6. The method of making a composite flint of a pyrophoric alloy and a protective covering which comprises casting the pyrophoric alloy into the form of a rod, enclosing the cast rod in a snugly fitting metallic sheath to form a composite ingot, working the composite ingot to a desired shape by a cold working process, and cutting the rod to desired lengths.

7. The method of making a composite flint of a pyrophoric alloy and a protective covering which comprises casting the pyrophoric alloy into the form of a rod, enclosing the cast rod in a snugly fitting metallic sheath to form a composite ingot, reducing the composite ingot to form a rod of desired shape by hot working followed by cold working, removing a portion of the enclosing sheath from the rod to expose the pyrophoric alloy, and cutting the rod to desired lengths.

8. The method of making a composite flint of a pyrophoric cerium alloy and a protective metallic covering which comprises casting the pyrophoric alloy into the form of a rod, enclosing the cast rod in a snugly fitting metallic sheath to form a composite article, reducing the composite article thus formed by hot rolling followed with cold rolling, and removing a portion of the enclosing sheath to expose the pyrophoric alloy.

CHARLES H. VAN DUSEN, JR.  
EDWIN C. DIETRICH.